

# UNITED STATES PATENT OFFICE.

THOMAS HARRIS AND CHARLES DAY, OF XENIA, OHIO.

## INCRUSTATION PREVENTIVE.

SPECIFICATION forming part of Letters Patent No. 410,516, dated September 3, 1889.

Application filed October 22, 1888. Serial No. 288,841. (No specimens.)

*To all whom it may concern:*

Be it known that we, THOMAS HARRIS and CHARLES DAY, of the city of Xenia, in the county of Greene and State of Ohio, have 5 invented certain new and useful Improvements in Compositions for Removing Scale from Steam-Boilers; and we do hereby declare that the following is a full, clear, and exact description thereof.

10 This invention is a composition for use in steam-boilers to prevent the formation of "scale" therein and to remove such scale if formed. The composition, when mixed with the water in or to be fed into the boiler, as 15 hereinafter stated, will effectually "break" the water or prevent its foaming or depositing sediment on the boiler-tubes.

The composition consists of the following ingredients, in or about the proportions 20 stated: one gallon of coal-oil, one pint of black oil, one ounce of flour, (wheat,) one ounce of lard. The "black oil" referred to is the oil produced in West Virginia, or lubricating-oil, not a good illuminant. By "coal- 25 oil" is meant kerosene such as is produced in Pennsylvania, which is a good burning-oil. These ingredients are thoroughly commingled, and about a half-gallon of the mixture is used per week with a fifty-horse-power boiler 30 (larger boilers in proportion) until all the scales have been removed, when the quantity

may be lessened. This composition has been tested and has been found effective in cleansing and preventing scale.

The office of the lard, flour, and black oil 35 is to form a gloss on the shell of the boiler and prevent further deposits clinging or sticking thereto, and also prevent fomenting of the water, while the coal-oil cuts off any scale that had previously formed. The black oil 40 (West Virginia oil) will not cut the scale alone, but requires the presence of the stronger and more penetrating petroleum or coal oil. The lard and flour assist in forming and keeping the preservative coating on the shell. 45

Having described our invention, we claim—  
The herein-described composition for removing scale from steam-boilers, consisting of one gallon of coal-oil, one pint of black oil, one ounce of wheat-flour, and one ounce of 50 lard, as and for the purpose set forth.

In testimony that we claim the foregoing as our own we affix our signatures in presence of two witnesses.

THOMAS + HARRIS.  
mark

CHARLES + DAY.  
mark

Witnesses:

ABNER S. BUCK,  
CHAS. S. BUCK.